

## UNITED STATES PATENT OFFICE.

GUSTAV GOLDMAN, OF BALTIMORE, MARYLAND.

## PROCESS OF MATTING OR FELTING FIBERS TOGETHER.

SPECIFICATION forming part of Letters Patent No. 758,243, dated April 26, 1904.

Application filed August 29, 1903. Serial No. 171,288. (No specimens.)

*To all whom it may concern:*

Be it known that I, GUSTAV GOLDMAN, of Baltimore, Maryland, have invented a new and useful Process of Matting or Felting Fibers Together, which invention is fully set forth 5 in the following specification.

This invention relates to the art of treating fibrous material for the purpose of uniting the fibers into a mass.

10 The felting of wool and hair or of the admixture of these fibers with other animal and vegetable fibers is dependent upon the natural physical properties of wool and hair, although the resulting fabric is given a subsequent treatment with a liquid sizing to invest it with certain specific properties, such as stiffness, hardness, or surface characteristics. Nevertheless felting processes in the present state of the art are inapplicable to fiber of vegetable or mineral origin unless wool and hair be introduced as the felting agent. There are many objections to the felting operation even of wool and hair or the admixture of wool and hair with other fibers as they are now 15 manufactured, among which may be mentioned the difficulty of producing a sheet or mass of uniform and even thickness throughout and of uniform structure; but the most important consideration is the unavoidable 20 and serious shrinkage invariably associated with present felting methods.

The object of the present invention is to provide a method of treating fibrous materials of any character, whether animal, vegetable, or 25 mineral or mixtures of these or any of these, so as to produce a sheet or mass of such fibers which shall cohere or be united together with any desired degree of compactness and tenacity.

30 With this object in view the invention, broadly stated, consists in the introduction between the fibers to be treated of any suitable binding material in a dry and finely-divided state, the binding material being of such character that in the presence of a suitable solvent or as the result of subsequent treatment or chemical reaction or by reason of its inherent properties it serves to bind the fibers together. Preferably the fibers are in a more or less 35 40 45 50 loose or fluffy condition when the dry finely-

divided material is applied to or introduced between the fibers, and it is therefore able to uniformly penetrate or sift into the fibrous mass and come into contact with individual fibers thereof. This is due to the fact that the binding material at the time of its introduction is in the form of powder or other finely-divided state, whereby it is enabled to be more uniformly applied and distributed, and to the further fact that at the time of its application or introduction it is in such condition that it does not adhere to the machinery or cause the material under treatment to adhere to the operating machinery. This condition is herein described as a "dry" condition and is meant to include any and all conditions of the binding material or materials which will permit it or them to be introduced between the fibers in a finely-divided state, preferably as a powder or similar state of fine division. While the powdered form of the binder is preferred in order that it may sift in between the fibers, this is not essential, as the binder may be, if desired, and in some instances is finely divided into infinitesimally thin sheets or into minute threads which are introduced between films or layers of the fibers or otherwise.

From the foregoing description it will be evident that for the purposes of this invention it is not essential that the binding material should actually sift through the entire mass of the fibers under treatment. It is equally within the invention if the binding material be applied to those fibers lying near the exterior surface or surfaces of the mass of fibers under treatment or if the binding material operates upon successive superimposed films or sheets, so as to bind the fibers together into a combined felted mass.

90 The broad inventive idea may find expression in a great variety of forms. Thus the binding material may be either a single material or it may be a mixture of two or more materials. It may be a material requiring the mechanical introduction of a suitable solvent or the application of heat to place it in condition to bind the fibers together, or by reason of the inherent qualities of such binding material or materials a binding condition may be 95 100

obtained without the mechanical introduction of the solvent. For example, dry dextrine may be used as the binding material and moisture in the form of steam or vapor after-  
ward applied mechanically, or a binder, as gelatin or glue, may be applied together with a deliquescent substance, as magnesium chlo-  
rid, the moisture necessary to dissolve the binding material being supplied through the  
agency of the deliquescent salt. Again, a binder, as starch, flour, &c., may be introduced together with a substance containing water chemically held—as, for example, crystalline sodium carbonate—the moisture necessary to render the binder operative being obtained by expelling through heat or otherwise the water from such water-containing substances. In still another form of the invention the material which is to constitute the binding agent  
may be introduced among the fibers in the form of two or more substances in a finely-  
divided condition, said substances being of such character that they will react or may be caused to react and produce a new substance which binds the fibers together. Thus a soluble soap, as soda-soap, and a salt of a suitable metal, as sulfate of zinc, may be introduced among the fibers separately or mixed together and subsequently treated, for example, by steam, thus causing the metal of the salt to unite with the soap and form an insoluble metallic soap which will constitute a waterproof binder for the fibers. In this instance the soluble soap would itself constitute a binder; but its value as a binding agent is inferior to that of the insoluble metallic soap resulting from the chemical reaction between the soluble soap and the metallic salt. Again, a binding material—as, for example, glue or gelatin—may be introduced together with an appropriate substance having no functions as a binder—as, for example, a salt of chrome or aluminium—but which will render such binding material subsequently insoluble, and therefore waterproof.

From the foregoing it will be understood that generically stated the invention consists in introducing between the fibers a material in a dry pulverulent or other finely-divided form, which material subsequently, as the result of mechanical treatment or chemical reaction or otherwise, becomes an active and efficient binding agent. The treatment necessary to render the material actively efficient as a binding agent may consist in supplying a solvent in the form of steam, vapor, gas, or otherwise, depending upon the particular binder employed, or the solvent may be supplied by the use of a deliquescent or other hygroscopic salt or a substance containing water chemically held, or instead of supplying a solvent to any particular binding agent chemical reaction between a plurality of substances may be relied upon to supply the binder, or the material may be rendered ac-

tively efficient as a binding agent by mechanical treatment—as, for instance, by heat. The specific method which it is best to employ will be determined by the kind of fibers used, the use to which the treated fibers are to be put, the cost of materials, &c. One specific method of procedure which has given very satisfactory results is as follows: The fiber to be treated—say cotton for example—is disposed in a suitable film by the carding-machine, and the appropriate binding material—for instance, ordinary gelatin or glue and magnesium chlorid—are dusted between the fibers, preferably as they come from the carding-machines, or between successive superimposed films. The fibrous material is then subjected to heat and pressure, preferably in the presence of steam, and for mechanical convenience, continuity of operation, and economy of production the fabric into which the appropriate binding material has been introduced, as hereinbefore indicated, is carried between heated rollers. The result of this treatment is to render the gelatin or glue capable of effectively binding the cotton into a felt or matted mass. With cotton fiber other binding substances may be used with equally satisfactory results, and for wool or other animal fiber and for mineral or vegetable fiber different binding materials will naturally suggest themselves as more economical, convenient, and satisfactory, and the combination of the characteristics of the fiber and of the binding material used will determine whether the active binding is to be accomplished by dissolving the binding material or by chemical reaction or by mechanical treatment or otherwise.

From the foregoing it will be perceived that the present invention provides a method for efficiently binding any character of fibrous material into a compact mass, which method is readily practiced by the use of automatic machinery or by hand, using cheap but highly effective binding materials, which may be easily and uniformly applied. This renders possible the economical production of a uniform product possessing in a high degree all those properties essential in padding and a great variety of other uses.

With many forms of binding material capable of use in practicing the invention the use of steam is extremely desirable if the very best results are to be secured, though the invention can be successfully practiced in a variety of forms without the use of steam. When steam is used, it may be either formed without the mass of fibers and then forced or caused to penetrate therethrough, or moisture may be introduced among the fibers by means of a moisture-bearing substance—a deliquescent or other hygroscopic substance, an efflorescent substance, or otherwise—and then the moisture converted into steam by supplying heat above 212° Fahrenheit, or, if desired, 130

a moisture-bearing substance may be introduced and steam from an external source also supplied.

For the purpose of clearly demonstrating the character and scope of the invention generically several specific methods have been disclosed herein, some of which have not been specifically claimed, though they are intended to be covered by the generic claims. These several specific methods not claimed herein will form the subject-matter of separate applications.

Having thus described the invention, what is claimed is—

15 1. The method of binding fibers together, which consists in introducing between the fibers a binding material or materials in dry form, and then treating said materials so as to make them an active binder.

20 2. The method of binding fibers together which consists in introducing between the fibers a dry finely-divided substance as a binder, and treating said finely-divided substance with another substance which will render it an active binder.

25 3. The method of treating fibers or fibrous material which consists in introducing between the fibers a dry finely-divided binding material, and then treating said binding material with a solvent thereof, whereby it is rendered capable of actively binding the fibers together.

35 4. The method of treating fibers or fibrous material which consists in introducing between the fibers a dry finely-divided binding material, and then treating said binding material with a solvent thereof, whereby it is rendered capable of actively binding the fibers together, and then driving off the solvent.

40 5. The method of treating fibers or fibrous material, which consists in introducing between the fibers a dry finely-divided binding material together with a substance capable of imparting moisture to said binding material, whereby it is rendered capable of actively binding the fibers together.

45 6. The method of treating fibers or fibrous material which consists in introducing between the fibers a dry finely-divided binding material together with a substance capable of imparting moisture to said binding material, whereby it is rendered capable of actively binding the fibers together, and then driving off the moisture.

55 7. The method of treating fibers or fibrous material which consists in introducing between the fibers a dry finely-divided binding material together with a hygroscopic substance, whereby moisture will be imparted to the binding material and it will be rendered capable of actively binding the fibers together.

8. The method of treating fibers or fibrous material which consists in introducing between the fibers a dry finely-divided binding material together with a hygroscopic substance,

whereby moisture will be imparted to the binding material and it will be rendered capable of actively binding the fibers together, and then driving off the moisture.

9. The method of treating fibers or fibrous material which consists in introducing between the fibers a dry finely-divided binding material together with a deliquescent substance, whereby moisture will be imparted to the binding material and it will be rendered capable of actively binding the fibers together.

10. The method of treating fibers or fibrous material which consists in introducing between the fibers a dry finely-divided binding material together with a deliquescent substance, whereby moisture will be imparted to the binding material and it will be rendered capable of actively binding the fibers together.

11. The method of treating fibers or fibrous material which consists in introducing between the fibers dry finely-divided gelatin together with a hygroscopic material, whereby moisture will be imparted to the gelatin and it will be rendered capable of actively binding the fibers together.

12. The method of treating fibers or fibrous material which consists in introducing between the fibers dry finely-divided gelatin together with a deliquescent material, whereby moisture will be imparted to the gelatin and it will be rendered capable of actively binding the fibers together.

13. The method of treating fibers or fibrous material which consists in introducing between the fibers dry finely-divided gelatin together with magnesium chlorid, whereby moisture will be imparted to the gelatin and it will be rendered capable of binding the fibers together.

14. The method of treating fibers or fibrous material which consists in introducing between the fibers dry finely-divided binding material, treating said binding material with a solvent thereof, and then subjecting the fibers to pressure.

15. The method of treating fibers or fibrous material which consists in introducing between the fibers dry finely-divided binding material, treating said binding material with a solvent thereof, and then subjecting the fibers to heat and pressure.

16. The method of treating fibers or fibrous material which consists in introducing between the fibers dry finely-divided binding material together with a substance capable of imparting moisture to said binding material and then subjecting the fibers to pressure.

17. The method of treating fibers or fibrous material which consists in introducing between the fibers dry finely-divided binding material together with a substance capable of imparting moisture to said binding material, and then subjecting the fibers to heat and pressure.

18. The method of treating fibers or fibrous

- material which consists in introducing between the fibers dry finely-divided binding material together with a hygroscopic substance, whereby moisture will be imparted to said binding material and it will be rendered capable of actively binding the fibers together, and then subjecting said fibers to pressure.
19. The method of treating fibers or fibrous material which consists in introducing between the fibers dry finely - divided binding material together with a hygroscopic substance, whereby moisture will be imparted to said binding material and it will be rendered capable of actively binding the fibers together, and then subjecting said fibers to heat and pressure.
20. The method of treating fibers or fibrous material which consists in introducing between the fibers dry finely - divided binding material together with a deliquescent substance, whereby moisture will be imparted to said binding material and it will be rendered capable of actively binding the fibers together, and then subjecting said fibers to pressure.
21. The method of treating fibers or fibrous material which consists in introducing between the fibers dry finely-divided binding material together with a deliquescent substance, whereby moisture will be imparted to said binding material and it will be rendered capable of actively binding the fibers together, and then subjecting said fibers to heat and pressure.
22. The method of treating fibers or fibrous material which consists in introducing between the fibers dry finely - divided gelatin together with a hygroscopic material, whereby moisture will be imparted to the gelatin and it will be rendered capable of actively binding the fibers together, and then subjecting the fibers to pressure.
23. The method of treating fibers or fibrous material which consists in introducing between the fibers dry finely - divided gelatin together with a hygroscopic material, whereby moisture will be imparted to the gelatin and it will be rendered capable of actively binding the fibers together, and then subjecting the fibers to heat and pressure.
24. The method of treating fibers or fibrous material which consists in introducing between the fibers dry finely-divided gelatin together with a deliquescent material, whereby moisture will be imparted to the gelatin and it will be rendered capable of actively binding the fibers together, and then subjecting the fibers to pressure.
25. The method of treating fibers or fibrous material which consists in introducing between the fibers dry finely-divided gelatin together with a deliquescent material, whereby moisture will be imparted to the gelatin and it will be rendered capable of actively binding the fibers together, and then subjecting the fibers to heat and pressure.
26. The method of treating fibers or fibrous material which consists in introducing between the fibers dry finely-divided binding material together with magnesium chlorid, whereby moisture will be imparted to the binding material and it will be rendered capable of binding the fibers together.
27. The method of treating fibers or fibrous material which consists in introducing between the fibers dry finely-divided binding material together with magnesium chlorid, whereby moisture will be imparted to the binding material and it will be rendered capable of binding the fibers together, and then subjecting the fibers to pressure.
28. The method of treating fibers or fibrous material which consists in introducing between the fibers dry finely-divided binding material together with magnesium chlorid, whereby moisture will be imparted to the binding material and it will be rendered capable of binding the fibers together, and then subjecting the fibers to heat and pressure.
29. The method of treating fibers or fibrous material which consists in introducing between the fibers dry finely-divided gelatin together with magnesium chlorid, whereby moisture will be imparted to the gelatin and it will be rendered capable of binding the fibers together, and then subjecting the fibers to pressure.
30. The method of treating fibers or fibrous material which consists in introducing between the fibers dry finely-divided gelatin together with magnesium chlorid, whereby moisture will be imparted to the gelatin and it will be rendered capable of binding the fibers together, and then subjecting the fibers to heat and pressure.
- In testimony whereof I have signed this specification in the presence of two subscribing witnesses.
- GUSTAV GOLDMAN.
- Witnesses:
- ARTHUR LEE BROWNE,  
FRANCIS T. HOMER.